



US006137516A

# United States Patent [19]

Malhotra et al.

[11] Patent Number: 6,137,516

[45] Date of Patent: \*Oct. 24, 2000

[54] RECORDING SHEETS CONTAINING  
MILDEW PREVENTING AGENTS[75] Inventors: **Shadi L. Malhotra**, Mississauga; **Brent S. Bryant**, Milton; **Arthur Y. Jones**, Mississauga, all of Canada[73] Assignee: **Xerox Corporation**, Stamford, Conn.

[ \* ] Notice: This patent is subject to a terminal disclaimer.

[21] Appl. No.: **08/504,266**[22] Filed: **Jul. 19, 1995**

## Related U.S. Application Data

[62] Division of application No. 08/196,605, Feb. 15, 1994, Pat. No. 5,663,004.

[51] **Int. Cl.**<sup>7</sup> ..... **B41M 5/00**; B41J 2/01[52] **U.S. Cl.** ..... **347/105**; 428/195[58] **Field of Search** ..... 428/195; 347/105

[56]

## References Cited

### U.S. PATENT DOCUMENTS

|           |         |                       |         |
|-----------|---------|-----------------------|---------|
| 4,592,954 | 6/1986  | Malhotra .....        | 428/335 |
| 4,650,808 | 3/1987  | May et al. .....      | 514/372 |
| 4,865,914 | 9/1989  | Malhotra .....        | 428/331 |
| 5,073,448 | 12/1991 | Vieira et al. .....   | 428/195 |
| 5,129,948 | 7/1992  | Breton et al. .....   |         |
| 5,212,008 | 5/1993  | Malhotra et al. ..... | 428/216 |
| 5,254,403 | 10/1993 | Malhotra .....        | 428/323 |
| 5,254,421 | 10/1993 | Coppens .....         |         |
| 5,292,776 | 3/1994  | Donofrio et al. ..... | 33/18   |
| 5,451,458 | 9/1995  | Malhotra .....        | 428/195 |
| 5,451,466 | 9/1995  | Malhotra .....        | 428/195 |

Primary Examiner—Pamela R. Schwartz  
Attorney, Agent, or Firm—Judith L. Byorick

[57]

## ABSTRACT

Disclosed is a recording sheet which comprises a substrate, an image receiving coating, and a biocide.

**25 Claims, No Drawings**

## RECORDING SHEETS CONTAINING MILDEW PREVENTING AGENTS

This is a division of application Ser. No. 08/196,605, filed Feb. 15, 1994 now U.S. Pat. No. 5,663,004.

### BACKGROUND OF THE INVENTION

The present invention is directed to recording sheets suitable for use in printing processes. More specifically, the present invention is directed to recording sheets and processes for the use thereof, wherein the recording sheet is resistant to mildew in high humidity environments. One embodiment of the present invention is directed to a recording sheet which comprises a substrate, an image receiving coating, and a biocide.

Recording sheets, especially transparencies intended for use with aqueous inks, frequently comprise a substrate coated with a hydrophilic ink receiving layer which is of a material or a mixture of materials exhibiting good film forming characteristics as well as the ability to dry images in relatively short times, the capability of spreading dyes prior to drying, resistance to fingerprints, or other desirable characteristics. For example, U.S. Pat. No. 4,592,954 (Malhotra), the disclosure of which is totally incorporated herein by reference, discloses a transparency for ink jet printing which comprises a supporting substrate and thereover a coating consisting essentially of a blend of carboxymethyl cellulose and polyethylene oxides. Also disclosed are papers for use in ink jet printing comprising a plain paper substrate and a coating thereover consisting essentially of polyethylene oxides.

In addition, U.S. Pat. No. 4,865,914 (Malhotra), the disclosure of which is totally incorporated herein by reference, discloses a transparency which comprises a supporting substrate and thereover a blend comprising poly(ethylene oxide) and carboxy methyl cellulose together with a component selected from the group consisting of (1) hydroxypropyl cellulose; (2) vinylmethyl ether/maleic acid copolymer; (3) carboxymethyl hydroxyethyl cellulose; (4) hydroxyethyl cellulose; (5) acrylamide/acrylic acid copolymer; (6) cellulose sulfate; (7) poly(2-acrylamido-2-methyl propane sulfonic acid); (8) poly(vinyl alcohol); (9) poly(vinyl pyrrolidone); and (10) hydroxypropyl methyl cellulose. In addition, papers with the aforementioned coatings are disclosed.

U.S. Pat. No. 5,212,008 (Malhotra et al.), the disclosure of which is totally incorporated herein by reference, discloses a recording sheet which comprises a substrate; a first coating in contact with the substrate which comprises a crosslinking agent selected from the group consisting of hexamethoxymethyl melamine, methylated melamine-formaldehyde, methylated urea-formaldehyde, cationic urea-formaldehyde, cationic polyamine-epichlorohydrin, glyoxal-urea resin, poly(aziridine), poly(acrylamide), poly(N,N-dimethyl acrylamide), acrylamide-acrylic acid copolymer, poly(2-acrylamido-2-methyl propane sulfonic acid), poly(N,N-dimethyl-3,5-dimethylene piperidinium chloride), poly(methylene-guanidine) hydrochloride, poly(ethylene imine) poly(ethylene imine) epichlorohydrin, poly(ethylene imine) ethoxylated, glutaraldehyde, and mixtures thereof; a catalyst; and a polymeric material capable of being crosslinked by the crosslinking agent and selected from the group consisting of polysaccharides having at least one hydroxy group, polysaccharides having at least one carboxy group, polysaccharides having at least one sulfate group, polysaccharides having at least one amine or amino group,

polysaccharide gums, poly(alkylene oxides), vinyl polymers, and mixtures thereof; and a second coating in contact with the first coating which comprises a binder and a material selected from the group consisting of fatty imidazolines, ethosulfate quaternary compounds, dialkyl dimethyl methosulfate quaternary compounds, alkoxylated di-fatty quaternary compounds, amine oxides, amine ethoxylates, Imidazoline quaternary compounds, alkyl benzyl dimethyl quaternary compounds, poly(epiamines), and mixtures thereof.

U.S. Pat. No. 5,254,403 (Malhotra), the disclosure of which is totally incorporated herein by reference, discloses a recording sheet which comprises a substrate and an image receiving layer comprising a mixture of (a) a polymer capable of forming a latex and selected from the group consisting of poly(vinyl chloride), ethylene-vinyl chloride copolymers, poly(vinyl acetate), carboxylated poly(vinyl acetate), ethylene-vinyl acetate copolymers, polymers containing acrylate monomers, polystyrene, styrene-butadiene copolymers, carboxylated styrene-butadiene copolymers, butadiene-acrylonitrile copolymers, butadiene-acrylonitrile-styrene copolymers, and mixtures thereof; (b) a polysaccharide; and (c) a polymer containing oxyalkylene monomers.

Copending application U.S. Ser. No. 08/196,669, with the named inventors Shadi L. Malhotra, Kurt B. Gundlach, and Richard L. Colt, filed concurrently herewith, entitled "Recording Sheets for Printing Processes Using Microwave Drying," now U.S. Pat. No. 5,663,004, the disclosure of which is totally incorporated herein by reference, discloses a printing process which comprises (a) providing a recording sheet which comprises a substrate, at least one monomeric salt, an optional binder, an optional antistatic agent, an optional biocide, and an optional filler; (b) applying an aqueous recording liquid to the recording sheet in an image-wise pattern; and (c) thereafter exposing the substrate to microwave radiation, thereby drying the recording liquid on the recording sheet.

Copending application U.S. Ser. No. 08/196,922, with the named inventor Shadi L. Malhotra, filed concurrently herewith, entitled "Recording Sheets Containing Alcohols and Saccharides," the disclosure of which is totally incorporated herein by reference, discloses a recording sheet which comprises a substrate and a material selected from the group consisting of monosaccharides, oligosaccharides, and mixtures thereof. Another embodiment of the present invention is directed to a printing process which comprises (a) providing a recording sheet which comprises a substrate, a material selected from the group consisting of monomeric alcohols, monosaccharides, oligosaccharides, and mixtures thereof, an optional binder, an optional antistatic agent, an optional biocide, and an optional filler; (b) applying an aqueous recording liquid to the recording sheet in an image-wise pattern; and (c) thereafter exposing the substrate to microwave radiation, thereby drying the recording liquid on the recording sheet.

Copending application U.S. Ser. No. 08/196,922, with the named inventor Shadi L. Malhotra, filed concurrently herewith, entitled "Recording Sheets," now U.S. Pat. No. 5,451,466 the disclosure of which is totally incorporated herein by reference, discloses a recording sheet which comprises (a) a substrate; (b) a coating on the substrate which comprises (i) a binder selected from the group consisting of (A) copolymers of styrene and at least one other monomer; (B) copolymers containing acrylic monomers and at least one other monomer; and (C) mixtures thereof; and (ii) an additive having a melting point of less than about 65° C. and a boiling point of more than about 150° C. and

selected from the group consisting of (A) diphenyl compounds; (B) phenyl alkanes; (C) indan compounds; (D) benzene derivatives; (E) benzyl alcohols; (F) phenyl alcohols; (G) menthol; (H) aromatic amines; and (I) mixtures thereof; (c) an optional filler; (d) an optional antistatic agent; and (e) an optional biocide. Also disclosed is a process for generating images which comprises (1) generating an electrostatic latent image on an imaging member in an imaging apparatus; (2) developing the latent image with a toner which comprises a colorant and a resin selected from the group consisting of (A) copolymers of styrene and at least one other monomer; (B) copolymers containing acrylic monomers and at least one other monomer; and (C) mixtures thereof; and (3) transferring the developed image to a recording sheet which comprises (a) a substrate; (b) a coating on the substrate which comprises (i) a polymeric binder selected from the group consisting of (A) copolymers of styrene and at least one other monomer; (B) copolymers containing acrylic monomers and at least one other monomer; and (C) mixtures thereof; and (ii) an additive having a melting point of less than about 65° C. and a boiling point of more than about 150° C. and selected from the group consisting of (A) diphenyl compounds; (B) phenyl alkanes; (C) indan compounds; (D) benzene derivatives; (E) benzyl alcohols; (F) phenyl alcohols; (G) menthol; (H) aromatic amines; (I) aliphatic amines; (J) aldehydes; (K) aldehyde derivatives; and (L) mixtures thereof; (c) an optional filler; (d) an optional antistatic agent; and (e) an optional biocide.

Copending application U.S. Ser. No. 08/196,673, with the named inventor Shadi L. Malhotra, filed concurrently herewith, entitled "Recording Sheets," the disclosure of which is totally incorporated herein by reference, now U.S. Pat. No. 5,451,458 discloses a recording sheet which comprises (a) a substrate; (b) a coating on the substrate which comprises (1) a binder selected from the group consisting of (A) polyesters; (B) polyvinyl acetals; (C) vinyl alcohol-vinyl acetal copolymers; (D) polycarbonates; and (E) mixtures thereof; and (2) an additive having a melting point of less than about 65° C. and a boiling point of more than about 150° C. and selected from the group consisting of (1) furan derivatives; (2) cyclic ketones; (3) lactones; (4) cyclic alcohols; (5) cyclic anhydrides; (6) acid esters; (7) phosphine oxides; and (8) mixtures thereof; (c) an optional filler; (d) an optional antistatic agent; and (e) an optional biocide. Also disclosed is a process for generating images which comprises (1) generating an electrostatic latent image on an imaging member in an imaging apparatus; (2) developing the latent image with a toner which comprises a colorant and a resin selected from the group consisting of (A) polyesters; (B) polyvinyl acetals; (C) vinyl alcohol-vinyl acetal copolymers; (D) polycarbonates; and (E) mixtures thereof; and (3) transferring the developed image to a recording sheet which comprises (a) a substrate; (b) a coating on the substrate which comprises (1) a binder selected from the group consisting of (A) polyesters; (B) polyvinyl acetals; (C) vinyl alcohol-vinyl acetal copolymers; (D) polycarbonates; and (E) mixtures thereof; and (2) an additive having a melting point of less than about 65° C. and a boiling point of more than about 150° C. and selected from the group consisting of (1) furan derivatives; (2) cyclic ketones; (3) lactones; (4) cyclic alcohols; (5) cyclic anhydrides; (6) acid esters; (7) esters; (8) phenones; (9) phosphine oxides; and (10) mixtures thereof; (c) an optional filler; (d) an optional antistatic agent; and (e) an optional biocide.

Copending application U.S. Ser. No. 08/196,679, with the named inventor Shadi L. Malhotra, filed concurrently herewith, entitled "Recording Sheets Containing Amino

Acids, Hydroxy Acids, and Polycarboxyl Compounds," now U.S. Pat. No. 5,589,277, the disclosure of which is totally incorporated herein by reference, discloses a recording sheet which comprises a paper substrate and a material selected from the group consisting of monomeric amino acids, monomeric hydroxy acids, monomeric polycarboxyl compounds, and mixtures thereof. Another embodiment of the present invention is directed to a recording sheet which comprises a paper substrate and an additive material selected from the group consisting of monomeric amino acids, monomeric hydroxy acids, monomeric polycarboxyl compounds, and mixtures thereof.

Copending application U.S. Ser. No. 08/196,607, with the named inventor Shadi L. Malhotra, filed concurrently herewith, entitled "Recording Sheets Containing Amine Salts and Quaternary Choline Halides," now U.S. Pat. No. 5,759,701, the disclosure of which is totally incorporated herein by reference, discloses a recording sheet which comprises a substrate and a material selected from the group consisting of monomeric amine acid salts, monomeric quaternary choline halides, and mixtures thereof.

Copending application U.S. Ser. No. 08/196,676, with the named inventor Shadi L. Malhotra, filed concurrently herewith, entitled "Recording Sheets Containing Pyrrole, Pyrrolidine, Pyridine, Piperidine, Homopiperidine, Quinoline, Isoquinoline, Quinuclidine, Indole, and Indazole Compounds," the disclosure of which is totally incorporated herein by reference, discloses a recording sheet which comprises a substrate and an additive material selected from the group consisting of pyrrole compounds, pyrrolidine compounds, pyridine compounds, piperidine compounds, homopiperidine compounds, quinoline compounds, isoquinoline compounds, quinuclidine compounds, indole compounds, indazole compounds, and mixtures thereof.

Copending application U.S. Ser. No. 08/196,933, with the named inventor Shadi L. Malhotra, filed concurrently herewith, entitled "Recording Sheets Containing Purine, Pyrimidine, Benzimidazole, Imidazolidine, Urazole, Pyrazole, Triazole, Benzotriazole, Tetrazole, and Pyrazine Compounds," the disclosure of which is totally incorporated herein by reference, discloses a recording sheet which comprises a substrate and a material selected from the group consisting of purine compounds, pyrimidine compounds, benzimidazole compounds, imidazolidine compounds, urazole compounds, pyrazole compounds, triazole compounds, benzotriazole compounds, tetrazole compounds, pyrazine compounds, and mixtures thereof. Also disclosed is a recording sheet which consists essentially of a substrate, at least one material selected from the group consisting of purine compounds, pyrimidine compounds, benzimidazole compounds, imidazolidine compounds, urazole compounds, pyrazole compounds, triazole compounds, benzotriazole compounds, tetrazole compounds, pyrazine compounds, and mixtures thereof, an optional binder, an optional antistatic agent, an optional biocide, and an optional filler.

Copending application U.S. Ser. No. 08/196,672, with the named inventor Shadi L. Malhotra, filed concurrently herewith, entitled "Recording Sheets Containing Oxazole, Isooxazole, Oxazolidinone, Oxazoline Salt, Morpholine, Thiazole, Thiazolidine, Thiadiazole, and Phenothiazine Compounds," the disclosure of which is totally incorporated herein by reference, discloses a recording sheet which comprises a substrate and a material selected from the group consisting of oxazole compounds, isooxazole compounds, oxazolidinone compounds, oxazoline salt compounds, morpholine compounds, thiazole compounds, thiazolidine compounds, thiadiazole compounds, phenothiazine

compounds, and mixtures thereof. Also disclosed is a recording sheet which consists essentially of a substrate, at least one material selected from the group consisting of oxazole compounds, isooxazole compounds, oxazolidinone compounds, oxazoline salt compounds, morpholine compounds, thiazole compounds, thiazolidine compounds, thiadiazole compounds, phenothiazine compounds, and mixtures thereof, an optional binder, an optional antistatic agent, an optional biocide, and an optional filler.

While suitable for their intended purposes, a need remains for improved recording sheets. In addition, a need remains for recording sheets which enable the formation of images which do not fade subsequent to drying of the sheet. Further, a need remains for recording sheets which enable the formation of images which are stable under high humidity conditions. Additionally, a need remains for recording sheets which exhibit long image quality and stability under a wide range of humidity conditions while also exhibiting resistance to attack by microorganisms. A need also remains for recording sheets which exhibit high image quality and stability as well as resistance to mildew when stored in plastic folders (such as polypropylene folders) under high humidity and/or heat conditions.

#### SUMMARY OF THE INVENTION

It is an object of the present invention to provide recording sheets with the above advantages.

It is another object of the present invention to provide improved recording sheets.

It is yet another object of the present invention to provide recording sheets which enable the formation of images which do not fade subsequent to drying of the sheet.

It is still another object of the present invention to provide recording sheets which enable the formation of images which are stable under high humidity conditions.

Another object of the present invention is to provide recording sheets which exhibit long image quality and stability under a wide range of humidity conditions while also exhibiting resistance to attack by microorganisms.

Yet another object of the present invention is to provide recording sheets which exhibit high image quality and stability as well as resistance to mildew when stored in plastic folders under high humidity and/or heat conditions.

These and other objects of the present invention (or specific embodiments thereof) can be achieved by providing a recording sheet which comprises a substrate, an image receiving coating, and a biocide.

#### DETAILED DESCRIPTION OF THE INVENTION

The recording sheets of the present invention comprise a substrate, an image receiving coating, and a biocide. Any suitable substrate can be employed. Examples include transparent materials, such as polyester, including Mylar™, available from E. I. Du Pont de Nemours & Company, Melinex™, available from Imperial Chemicals, Inc., Celanar™, available from Celanese Corporation, polyethylene naphthalates, such as Koladex PEN films, available from Imperial Chemicals, Inc., polycarbonates such as Lexan™, available from General Electric Company, polysulfones, such as those available from Union Carbide Corporation, polyether sulfones, such as those prepared from 4,4'-diphenyl ether, such as Udel™, available from Union Carbide Corporation, those prepared from disulfonyl chloride, such as Victrex™, available from ICI America Incorporated,

those prepared from biphenylene, such as Astrel™, available from 3M Company, poly (arylene sulfones), such as those prepared from crosslinked poly(arylene ether ketone sulfones), cellulose triacetate, polyvinylchloride cellophane, polyvinyl fluoride, polyimides, and the like, with polyester such as Mylar™ being preferred in view of its availability and relatively low cost. The substrate can also be opaque, including opaque plastics, such as Teslin™, available from PPG Industries, and filled polymers, such as Melinex®, available from ICI. Filled plastics can also be employed as the substrate, particularly when it is desired to make a "never-tear paper" recording sheet. Paper is also suitable, including plain papers such as Xerox® 4024, diazo papers, or the like.

In one embodiment of the present invention, the substrate comprises sized blends of hardwood kraft and softwood kraft fibers containing from about 10 to 90 percent by weight soft wood and from about 10 to about 90 percent by weight hardwood. Examples of hardwood include Seagull W dry bleached hardwood kraft, present in one embodiment in an amount of about 70 percent by weight. Examples of softwood include La Tuque dry bleached softwood kraft, present in one embodiment in an amount of about 30 percent by weight. These substrates can also contain fillers and pigments in any effective amounts, typically from about 1 to about 60 percent by weight, such as clay (available from Georgia Kaolin Company, Astro-fil 90 clay, Engelhard Ansilex clay), titanium dioxide (available from Tioxide Company—Anatase grade AHR), calcium silicate CH-427-97-8, XP-974 (J. M. Huber Corporation), and the like. The sized substrates can also contain sizing chemicals in any effective amount, typically from about 0.25 percent to about 25 percent by weight of pulp, such as acidic sizing, including Mon size (available from Monsanto Company), alkaline sizing such as Hercon-76 (available from Hercules Company), Alum (available from Allied Chemicals as Iron free alum), retention aid (available from Allied Colloids as Percol 292), and the like. The preferred internal sizing degree of papers selected for the present invention, including commercially available papers, varies from about 0.4 to about 5,000 seconds, and papers in the sizing range of from about 0.4 to about 300 seconds are more preferred, primarily to decrease costs. Preferably, the selected substrate is porous, and the porosity value of the selected substrate preferably varies from about 100 to about 1,260 milliliters per minute and preferably from about 50 to about 600 milliliters per minute to enhance the effectiveness of the recording sheet in ink jet processes. Preferred basis weights for the substrate are from about 40 to about 400 grams per square meter, although the basis weight can be outside of this range.

Illustrative examples of commercially available internally and externally (surface) sized substrates suitable for the present invention include Diazo papers, offset papers, such as Great Lakes offset, recycled papers, such as Conservatree, office papers, such as Automimeo, Eddy liquid toner paper and copy papers available from companies such as Nekoosa, Champion, Wiggins Teape, Kymmene, Modo, Domtar, Veitsiluoto and Sanyo, and the like, with Xerox® 4024™ papers and sized calcium silicate-clay filled papers being particularly preferred in view of their availability, reliability, and low print through. Pigmented filled plastics, such as Teslin (available from PPG industries), are also preferred as supporting substrates.

The substrate can be of any effective thickness. Typical thicknesses for the substrate are from about 50 to about 500 microns, and preferably from about 100 to about 125 microns, although the thickness can be outside these ranges.

Situated on the substrate of the present invention is an image receiving coating. Any suitable image receiving material can be employed. Examples of coating materials include (a) hydrophilic polysaccharides and their modifications, such as (1) starch (such as starch SLS-280, available from St. Lawrence starch), (2) cationic starch (such as Cato-72, available from National Starch), (3) hydroxyalkylstarch, wherein alkyl has at least one carbon atom and wherein the number of carbon atoms is such that the material is water soluble, preferably from about 1 to about 20 carbon atoms, and more preferably from about 1 to about 10 carbon atoms, such as methyl, ethyl, propyl, butyl, or the like (such as hydroxypropyl starch (#02382, available from Poly Sciences Inc.) and hydroxyethyl starch (#06733, available from Poly Sciences Inc.)), (4) gelatin (such as Calfskin gelatin #00639, available from Poly Sciences Inc.), (5) alkyl celluloses and aryl celluloses, wherein alkyl has at least one carbon atom and wherein the number of carbon atoms is such that the material is water soluble, preferably from 1 to about 20 carbon atoms, more preferably from 1 to about 10 carbon atoms, and even more preferably from 1 to about 7 carbon atoms, such as methyl, ethyl, propyl, butyl, pentyl, hexyl, benzyl, and the like (such as methyl cellulose (Methocel AM 4, available from Dow Chemical Company)), and wherein aryl has at least 6 carbon atoms and wherein the number of carbon atoms is such that the material is water soluble, preferably from 6 to about 20 carbon atoms, more preferably from 6 to about 10 carbon atoms, and even more preferably about 6 carbon atoms, such as phenyl, (6) hydroxy alkyl celluloses, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as hydroxyethyl cellulose (Natrosol 250 LR, available from Hercules Chemical Company), and hydroxypropyl cellulose (Klucel Type E, available from Hercules Chemical Company)), (7) alkyl hydroxy alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as ethyl hydroxyethyl cellulose (Bermocoll, available from Berol Kem. A.B. Sweden)), (8) hydroxy alkyl alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxyethyl methyl cellulose (HEM, available from British Celanese Ltd., also available as Tylose MH, MHK from Kalle A.G.), hydroxypropyl methyl cellulose (Methocel K35LV, available from Dow Chemical Company), and hydroxy butylmethyl cellulose (such as HBMC, available from Dow Chemical Company)), (9) dihydroxyalkyl cellulose, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dihydroxypropyl cellulose, which can be prepared by the reaction of 3-chloro-1,2-propane with alkali cellulose), (10) hydroxy alkyl hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxyethyl hydroxyethyl cellulose (Bermocoll, available from Berol Kem. A.B. Sweden)).

carbon atoms, such as methyl, ethyl, propyl, butyl and the like (such as hydroxypropyl hydroxyethyl cellulose, available from Aqualon Company), (11) halodeoxycellulose, wherein halo represents a halogen atom (such as chlorodeoxycellulose, which can be prepared by the reaction of cellulose with sulfuryl chloride in pyridine at 25° C.), (12) amino deoxycellulose (which can be prepared by the reaction of chlorodeoxy cellulose with 19 percent alcoholic solution of ammonia for 6 hours at 160° C.), (13) dialkylammonium halide hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as diethylammonium chloride hydroxy ethyl cellulose, available as Celquat H-100, L-200, National Starch and Chemical Company), (14) hydroxyalkyl trialkyl ammonium halide hydroxyalkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as hydroxypropyl trimethyl ammonium chloride hydroxyethyl cellulose, available from Union Carbide Company as Polymer JR), (15) dialkyl amino alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, (such as diethyl amino ethyl cellulose, available from Poly Sciences Inc. as DEAE cellulose #05178), (16) carboxyalkyl dextrans, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, and the like, (such as carboxymethyl dextrans, available from Poly Sciences Inc. as #16058), (17) dialkyl aminoalkyl dextran, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as diethyl aminoethyl dextran, available from Poly Sciences Inc. as #5178), (18) amino dextran (available from Molecular Probes Inc), (19) carboxy alkyl cellulose salts, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethyl cellulose CMC 7HOF, available from Hercules Chemical Company), (20) gum arabic (such as #G9752, available from Sigma Chemical Company), (21) carrageenan (such as #C1013 available from Sigma Chemical Company), (22) Karaya gum (such as #G0503, available from Sigma Chemical Company), (23) xanthan (such as Keltrol-T, available from Kelco division of Merck and Company), (24) chitosan (such as #C3646, available from Sigma Chemical Company), (25) carboxyalkyl hydroxyalkyl guar, wherein each alkyl has at least one carbon atom and wherein the number of carbon atoms is such that the material is water soluble, preferably from 1 to

about 20 carbon atoms, more preferably from 1 to about 10 carbon atoms, such as methyl, ethyl, propyl, butyl and the like (such as carboxymethyl hydroxypropyl guar, available from Auqualon Company), (26) cationic guar (such as Celanese Jaguars C-14-S, C-15, C-17, available from Celanese Chemical Company), (27) n-carboxyalkyl chitin, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, such as n-carboxymethyl chitin, (28) dialkyl ammonium hydrolyzed collagen protein, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dimethyl ammonium hydrolyzed collagen protein, available from Croda as Croquats), (29) agar-agar (such as that available from Pfaltz and Bauer Inc), (30) cellulose sulfate salts, wherein the cation is any conventional cation, such as sodium, lithium, potassium, calcium, magnesium, or the like (such as sodium cellulose sulfate #023 available from Scientific Polymer Products), and (31) carboxyalkylhydroxyalkyl cellulose salts, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethylhydroxyethyl cellulose CMHEC 43H and 37L available from Hercules Chemical Company); (b) vinyl polymers, such as (1) poly(vinyl alcohol) (such as Elvanol available from Dupont Chemical Company), (2) poly (vinyl phosphate) (such as #4391 available from Poly Sciences Inc.), (3) poly (vinyl pyrrolidone) (such as that available from GAF Corporation), (4) vinyl pyrrolidone-vinyl acetate copolymers (such as #02587, available from Poly Sciences Inc.), (5) vinyl pyrrolidone-styrene copolymers (such as #371, available from Scientific Polymer Products), (6) poly (vinylamine) (such as #1562, available from Poly Sciences Inc.), (7) poly (vinyl alcohol) alkoxylated, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl alcohol) ethoxylated #6573, available from Poly Sciences Inc.), and (8) poly (vinyl pyrrolidone-dialkylaminoalkyl alkylacrylate), wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl pyrrolidone-diethylaminomethylmethacrylate) #16294 and #16295, available from Poly Sciences Inc.); (c) formaldehyde resins, such as (1) melamine-formaldehyde resin (such as BC 309, available from British Industrial Plastics Limited), (2) urea-formaldehyde resin (such as BC777, available from British Industrial Plastics Limited), and (3) alkylated urea-formaldehyde resins, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methylated urea-formaldehyde resins, available

from American Cyanamid Company as Beetle 65); (d) ionic polymers, such as (1) poly (2-acrylamide-2-methyl propane sulfonic acid) (such as #175 available from Scientific Polymer Products), (2) poly (N,N-dimethyl-3,5-dimethylene piperidinium chloride) (such as #401, available from Scientific Polymer Products), and (3) poly (methylene-guanidine) hydrochloride (such as #654, available from Scientific Polymer Products); (e) latex polymers, such as (1) cationic, anionic, and nonionic styrene-butadiene latexes (such as that available from Gen Corp Polymer Products, such as RES 4040 and RES 4100, available from Unocal Chemicals, and such as DL 6672A, DL6638A, and DL6663A, available from Dow Chemical Company), (2) ethylene-vinylacetate latex (such as Airflex 400, available from Air Products and Chemicals Inc.), (3) vinyl acetate-acrylic copolymer latexes (such as synthemul 97-726, available from Reichhold Chemical Inc, Resyn 25-1110 and Resyn 25-1140, available from National Starch Company, and RES 3103 available from Unocal Chemicals; (4) quaternary acrylic copolymer latexes, particularly those of the formula



wherein n is a number of from about 10 to about 100, and preferably about 50, R is hydrogen or methyl, R<sub>1</sub> is hydrogen, an alkyl group, or an aryl group, and R<sub>2</sub> is N<sup>+</sup>(CH<sub>3</sub>)<sub>3</sub>X<sup>-</sup>, wherein X is an anion, such as Cl, Br, I, HSO<sub>3</sub>, SO<sub>3</sub>, CH<sub>2</sub>SO<sub>3</sub>, H<sub>2</sub>PO<sub>4</sub>, HPO<sub>4</sub>, PO<sub>4</sub>, or the like, and the degree of quaternization is from about 1 to about 100 percent, including polymers such as polymethyl acrylate trimethyl ammonium chloride latex, such as HX42-1, available from Interpolymer Corp., or the like; (f) maleic anhydride and maleic acid containing polymers, such as (1) styrene-maleic anhydride copolymers (such as that available as Scriptet from Monsanto, and the SMA series available from Arco), (2) vinyl alkyl ether-maleic anhydride copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinyl methyl ether-maleic anhydride copolymer #173, available from Scientific Polymer Products), (3) alkylene-maleic anhydride copolymers, wherein alkylene has at least one carbon atom and wherein the number of carbon atoms is such that the material is water soluble, preferably from 1 to about 10 carbon atoms, such as methyl, ethyl, propyl, butyl, and the like (such as ethylene-maleic anhydride copolymer #2308, available from Poly Sciences Inc., also available as EMA from Monsanto Chemical Company), (4) butadiene-maleic acid copolymers (such as #07787, available from Poly Sciences Inc.), (5) vinylalkylether-maleic acid copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinylmethylether-maleic acid copolymer, available from GAF Corporation as Gantrez S-95), and (6) alkyl vinyl ether-maleic acid esters, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methyl vinyl

ether-maleic acid ester #773, available from Scientific Polymer Products); (g) acrylamide containing polymers, such as (1) poly (acrylamide) (such as #02806, available from Poly Sciences Inc.), (2) acrylamide-acrylic acid copolymers (such as #04652, #02220, and #18545, available from Poly Sciences Inc.), and (3) poly (N,N-dimethyl acrylamide) (such as #004590, available from Poly Sciences Inc.); and (h) poly (alkylene imine) containing polymers, wherein alkylene has two (ethylene), three (propylene), or four (butylene) carbon atoms, such as (1) poly(ethylene imine) (such as #135, available from Scientific Polymer Products), (2) poly (ethylene imine) epichlorohydrin (such as #634, available from Scientific Polymer Products), and (3) alkoxyated poly (ethylene imine), wherein alkyl has one (methoxylated), two (ethoxylated), three (propoxylated), or four (butoxylated) carbon atoms (such as ethoxylated poly (ethylene imine) #636, available from Scientific Polymer Products); and the like, as well as blends or mixtures of any of the above, with starches and latexes being particularly preferred because of their availability and applicability to paper. Any mixtures of the above ingredients in any relative amounts can be employed.

In addition, the coating of the recording sheets of the present invention can contain optional antistatic agents. Any suitable or desired antistatic agent or agents can be employed, such as quaternary salts and other materials as disclosed in, for example, U.S. Pat. Nos. 5,760,809; 5,314,747; 5,441,795; 5,320,902; and 5,457,486, the disclosures of each of which are totally incorporated herein by reference. The antistatic agent can be present in any effective amount; typically, the antistatic agent is present in an amount of from about 1 to about 5 percent by weight of the coating, and preferably in an amount of from about 1 to about 2 percent by weight of the coating, although the amount can be outside these ranges.

Further, the coating of the recording sheets of the present invention can contain optional filler components. Fillers can be present in any effective amount, and if present, typically are present in amounts of from about 1 to about 60 percent by weight of the coating composition. Examples of filler components include colloidal silicas, such as Syloid 74, available from Grace Company (preferably present, in one embodiment, in an amount of about 20 weight percent), titanium dioxide (available as Rutile or Anatase from NL Chem Canada, Inc.), hydrated alumina (Hydrad TMC-HBF, Hydrad TM-HBC, available from J. M. Huber Corporation), barium sulfate (K.C. Blanc Fix HD80, available from Kali Chemie Corporation), calcium carbonate (Microwhite Sylacauga Calcium Products), high brightness clays (such as Engelhard Paper Clays), calcium silicate (available from J. M. Huber Corporation), cellulosic materials insoluble in water or any organic solvents (such as those available from Scientific Polymer Products), blend of calcium fluoride and silica, such as Opalex-C available from Kemira.O.Y, zinc oxide, such as Zoco Fax 183, available from Zo Chem, blends of zinc sulfide with barium sulfate, such as Lithopane, available from Schtебen Company, and the like, as well as mixtures thereof. Brightener fillers can enhance color mixing and assist in improving print-through in recording sheets of the present invention.

Situated in or on the image receiving coating is a biocide material. Any biocide which is capable of preventing mildew of the image receiving coating and which does not impair the quality and stability of the images produced thereon can be employed. The biocide can be present in any effective amount; typically, the biocide is present in an amount of from about 10 parts per million to about 3 percent by weight of the coating, although the amount can be outside this range.

Examples of suitable biocides include (A) non-ionic biocides, such as (1) 2-hydroxypropylmethane thiosulfonate (Busan 1005, available from Buckman Laboratories Inc.); (2) 2-(thio cyanomethyl thio) benzothiazole (Busan 30WB, 5 72WB, available from Buckman Laboratories Inc.); (3) methylene bis (thiocyanate) (Metasol T-10, available from Calgon Corporation; AMA-110, available from Vinings Chemical Company; Vichem MBT, available from Vineland Chemical Company; Aldrich 10,509-0); (4) 2-bromo-4'-hydroxyacetophenone (Busan 90, available from Buckman Laboratories); (5) 1,2-dibromo-2,4-dicyano-butane (Metasol CB-210, CB-235, available from Calgon Corporation); (6) 2,2-dibromo-3-nitropropionamide (Metasol RB-20, available from Calgon Corporation; Amerstat 300, available from Drew Industrial Div.); (7) N-~~■~~ -(1-nitroethyl benzylethylene diamine) (Metasol J-26, available from Calgon Corporation); (8) dichlorophene (G-4, available from Givaudan Corporation); (9) 3,5-dimethyl tetrahydro-2H-1,3,5-thiadiazine-2-thione (SLIME-TROL RX-28, available from Betz Paper Chem Inc.; Metasol D3T-A, available from Calgon Corporation; SLIME ARREST, available from Western Chemical Company); (10) a non-ionic blend of a sulfone, such as bis (trichloromethyl) sulfone and methylene bisthiocyanate (available as SLIME-TROL RX-38A from Betz Paper Chem Inc.); (11) a non-ionic blend of methylene bisthiocyanate and bromonitrostyrene (available as SLIME-TROL RX-41 from Betz Paper Chem Inc.); (12) a non-ionic blend of 2-(thiocyanomethylthio) benzothiazole (53.2% by weight) 20 and 2-hydroxypropyl methanethiosulfonate (46.8% by weight) (available as BUSAN 25 from Buckman Laboratories Inc.); (13) a non-ionic blend of methylene bis (thiocyanate) 50 percent by weight and 2-(thiocyanomethylthio) benzothiazole 50 percent by weight 25 (available as BUSAN 1009, 1009WB from Buckman Laboratories Inc.); (14) a non-ionic blend of 2-bromo-4'-hydroxyacetophenone (70 percent by weight) and 2-(thiocyanomethylthio) benzothiazole (30 percent by weight) (BUSAN 93, available from Buckman Laboratories Inc.); (15) a non-ionic blend of 5-chloro-2-methyl-4-isothiazoline-3-one (75 percent by weight) and 2-methyl-4-isothiazolin-3-one (25 percent by weight), (available as 30 AMERSTAT 250 from Drew Industrial Division; NALCON 7647, from NALCO Chemical Company;Kathon LY, from Rohm and Haas Co.); and the like, as well as mixtures thereof.

Also suitable are (B) anionic biocides, such as (1) anionic potassium N-hydroxymethyl-N-methyl-dithiocarbamate (available as BUSAN 40 from Buckman Laboratories Inc.); (2) an anionic blend of N-hydroxymethyl-N-methyl dithiocarbamate (80% by weight) and sodium 2-mercapto benzothiazole (20% by weight) (available as BUSAN 52 from Buckman Laboratories Inc.); (3) an anionic blend of sodium dimethyl dithiocarbamate 50 percent by weight and (disodium ethylenebisdithiocarbamate) 50% by weight (available as METASOL 300 from Calgon Corporation; AMERSTAT 272 from Drew Industrial Division; SLIME CONTROL F from Western Chemical Company); (4) an anionic blend of N-methyldithiocarbamate 60 percent by weight and disodium cyanodithioimidocarbonate 40 percent by weight (available as BUSAN 881 from Buckman Laboratories Inc); (5) An anionic blend of methylene bis-thiocyanate (33% by weight), sodium dimethyl-dithiocarbamate (33% by weight), and sodium ethylene bisdithiocarbamate (33% by weight) (available as AMERSTAT 282 from Drew Industrial Division; AMA-131 from Vinings Chemical Company); (6) sodium dichlorophene 45

(G-4-40, available from Givaudan Corp.); and the like, as well as mixtures thereof.

Also suitable are (C) cationic biocides, such as (1) cationic poly (oxyethylene (dimethylamino)-ethylene (dimethylamino) ethylene dichloride) (Busan 77, available from Buckman Laboratories Inc.); (2) a cationic blend of methylene bis thiocyanate and dodecyl guanidine hydrochloride (available as SLIME TROL RX-31, RX-32, RX-32P, RX-33, from Betz Paper Chem Inc.); (3) a cationic blend of a sulfone, such as bis(trichloromethyl) sulfone and a quaternary ammonium chloride (available as SLIME TROL RX-36 DPB-865 from Betz Paper Chem. Inc.); (4) a cationic blend of methylene bis thiocyanate and chlorinated phenols (available as SLIME-TROL RX-40 from Betz Paper Chem Inc.); and the like, as well as mixtures thereof.

The coating containing the biocide is present on the substrate of the recording sheet of the present invention in any effective thickness. Typically, the total thickness of the coating layer is from about 1 to about 25 microns and preferably from about 5 to about 10 microns, although the thickness can be outside of these ranges.

The image receiving coating containing the biocide (as well as the optional filler and/or optional antistatic agent, if present) can be applied to the substrate by any suitable technique, such as size press treatment, dip coating, reverse roll coating, extrusion coating, or the like. For example, the coating can be applied with a KRK size press (Kumagai Riki Kogyo Co., Ltd., Nerima, Tokyo, Japan) by dip coating and can be applied by solvent extrusion on a Faustel Coater. The KRK size press is a lab size press that simulates a commercial size press. This size press is normally sheet fed, whereas a commercial size press typically employs a continuous web. On the KRK size press, the substrate sheet is taped by one end to the carrier mechanism plate. The speed of the test and the roll pressures are set, and the coating solution is poured into the solution tank. A 4 liter stainless steel beaker is situated underneath for retaining the solution overflow. The coating solution is cycled once through the system (without moving the substrate sheet) to wet the surface of the rolls and then returned to the feed tank, where it is cycled a second time. While the rolls are being "wetted", the sheet is fed through the sizing rolls by pressing the carrier mechanism start button. The coated sheet is then removed from the carrier mechanism plate and is placed on a 12 inch by 40 inch sheet of 750 micron thick Teflon for support and is dried on the Dynamic Former drying drum and held under restraint to prevent shrinkage. The drying temperature is approximately 105° C. This method of coating treats both sides of the substrate simultaneously.

In dip coating, a web of the material to be coated is transported below the surface of the liquid coating composition by a single roll in such a manner that the exposed site is saturated, followed by removal of any excess coating by the squeeze rolls and drying at 100° C. in an air dryer. The liquid coating composition generally comprises the desired coating composition dissolved in a solvent such as water, methanol, or the like. The method of surface treating the substrate using a coater results in a continuous sheet of substrate with the coating material applied first to one side and then to the second side of this substrate. The substrate can also be coated by a slot extrusion process, wherein a flat die is situated with the die lips in close proximity to the web of substrate to be coated, resulting in a continuous film of the coating solution evenly distributed across one surface of the sheet, followed by drying in an air dryer at 100° C.

Recording sheets of the present invention can be employed in ink jet printing processes. One embodiment of

the present invention is directed to a process which comprises applying an aqueous recording liquid to a recording sheet of the present invention in an imagewise pattern. Another embodiment of the present invention is directed to a printing process which comprises (1) incorporating into an ink jet printing apparatus containing an aqueous ink a recording sheet of the present invention, and (2) causing droplets of the ink to be ejected in an imagewise pattern onto the recording sheet, thereby generating images on the recording sheet. Ink jet printing processes are well known, and are described in, for example, U.S. Pat. No. 4,601,777, U.S. Pat. No. 4,251,824, U.S. Pat. No. 4,410,899, U.S. Pat. No. 4,412,224, and U.S. Pat. No. 4,532,530, the disclosures of each of which are totally incorporated herein by reference. In a particularly preferred embodiment, the printing apparatus employs a thermal ink jet process wherein the ink in the nozzles is selectively heated in an imagewise pattern, thereby causing droplets of the ink to be ejected in image-wise pattern. In another preferred embodiment, the substrate is printed with an aqueous ink and thereafter the printed substrate is exposed to microwave radiation, thereby drying the ink on the sheet. Printing processes of this nature are disclosed in, for example, U.S. Pat. No. 5,220,346, the disclosure of which is totally incorporated herein by reference.

The recording sheets of the present invention can also be used in any other printing or imaging process, such as printing with pen plotters, handwriting with ink pens, offset printing processes, or the like, provided that the ink employed to form the image is compatible with the ink receiving layer of the recording sheet.

Specific embodiments of the invention will now be described in detail. These examples are intended to be illustrative, and the invention is not limited to the materials, conditions, or process parameters set forth in these embodiments. All parts and percentages are by weight unless otherwise indicated.

#### EXAMPLE I

Transparency sheets were prepared as follows. Blends of ink receptive coating materials and biocides as indicated in the Table below were prepared by mixing the materials in a 2 Liter jar and stirring the contents in an Omni homogenizer for 2 hours. Subsequently, the solution was left overnight for removal of air bubbles. The blends thus prepared were then coated by a dip coating process (both sides coated in one operation) by providing Mylar® base sheets in cut sheet form (8.5×11 inches) in a thickness of 100 microns. Subsequent to air drying at 100° C. for 10 minutes and monitoring the difference in weight prior to and subsequent to coating, the dried coated sheets were each coated with 1 gram, 10 microns in thickness, on each surface (2 grams total coating weight for 2-sided transparency) of the substrate.

The shelf lives of the transparencies thus prepared were measured by storing the sheets at 25° C. and 50 percent relative humidity and monitoring the development of white opaque mildew as a function of time. The transparencies prepared with non-ionic and anionic cellulosic rich coatings and not containing biocides (1 through 4 in the Table) developed mildew in about 4 to 6 months. In contrast, similar transparencies containing 1 percent by weight anionic sodium benzoate required a period of 10 months under the same conditions to exhibit the same degree of mildew development. The use of potassium N-hydroxymethyl-N-methyl dithiocarbamate was effective in prolonging the life of the transparency to 18 months, even at concentrations as low as 25 ppm by weight of the solids

content of the coating composition. In addition, the transparencies containing a blend of sodium-2-mercapto benzothiazole and potassium N-hydroxymethyl-N-methyl dithiocarbamate exhibited further increased shelf lives of 24 months. Further, the transparencies prepared with cationic ink receptive coatings, such as #9, and containing cationic blends of bis (trichloromethyl) sulfone and a quaternary ammonium chloride exhibited a shelf life of about 24 months. The transparencies prepared with non-ionic ink receptive coating compositions and non-ionic biocides (#10 and #11) also exhibited shelf lives of 24 months.

| #  | Coating Composition                                                                                                                                                                       | Biocide                                                                                                                                                            | Shelf life (mos.) |
|----|-------------------------------------------------------------------------------------------------------------------------------------------------------------------------------------------|--------------------------------------------------------------------------------------------------------------------------------------------------------------------|-------------------|
| 1  | hydroxypropylmethyl cellulose (HPMC) K35LV (Dow Chemicals), 6% by weight in water                                                                                                         | none                                                                                                                                                               | 6                 |
| 2  | sodium carboxymethyl cellulose CMC 7HOF (Hercules Chemicals), 1.5% by weight in water                                                                                                     | none                                                                                                                                                               | 6                 |
| 3  | hydroxypropylmethyl cellulose K35LV 75% by wt. and polyethylene oxide POLY OX WSRN-3000 25% by wt., 6% by weight in water                                                                 | none                                                                                                                                                               | 4                 |
| 4  | sodium carboxymethyl cellulose CMC 7HOF (Hercules Chemicals) 60% by wt. and polyethylene oxide POLY OX WSRN-3000 (Union Carbide) 40% by wt., 3% by weight in water                        | none                                                                                                                                                               | 4                 |
| 5  | same as 3                                                                                                                                                                                 | anionic sodium benzoate, 1% by wt.                                                                                                                                 | 10                |
| 6  | same as 4                                                                                                                                                                                 | anionic sodium benzoate, 1% by wt.                                                                                                                                 | 10                |
| 7  | same as 4                                                                                                                                                                                 | anionic potassium N-hydroxymethyl-N-methyl dithio carbamate Busan 40 (Buckman), 25 ppm by wt.                                                                      | 18                |
| 8  | same as 4                                                                                                                                                                                 | anionic blend of potassium N-hydroxymethyl-N-methyl dithiocarbamate (80% by wt.) and sodium 2-mercapto benzothiazole (20% by wt.) Busan 52 (Buckman) 25 ppm by wt. | 24                |
| 9  | cationic hydroxyethyl cellulose polymer JR-125 (Union Carbide) 75% by wt. and polyethylene oxide POLY OX WSRN-3000 25% by wt., 5% by weight in water                                      | cationic blend of bis (trichloromethyl) sulfone and a quaternary ammonium chloride SLIME TROL RX-36, 25 ppm by wt.                                                 | 24                |
| 10 | hydroxypropylmethyl cellulose (HPMC) K35LV 75% by wt. and Rhoplex B-15J acrylic latex (Rohm and Haas) 25% by wt., 25% by wt. in water                                                     | Kathon LX (Rohm and Haas) (nonionic blend of 5-chloro-2-methyl-4-isothiazolin-3-one and 2-methyl-4-isothiazolin-3-one) 25 ppm by wt.                               | 24                |
| 11 | anionic blend of hydroxypropylmethyl cellulose K35 LV 50% by wt., sodium carboxymethyl cellulose CMC 7HOF 25% by wt., polyethylene oxide POLY OX WSRN-3000 25% by wt., 4% by wt. in water | Busan 30 WB (Buckman) non-ionic 2-(thiocyanomethylthio) benzothiazole 25 ppm by wt.                                                                                | 24                |

Other embodiments and modifications of the present invention may occur to those skilled in the art subsequent to

a review of the information presented herein; these embodiments and modifications, as well as equivalents thereof, are also included within the scope of this invention.

What is claimed is:

- 5 1. A printing process which comprises (1) incorporating into an ink jet printing apparatus containing an aqueous ink a recording sheet which comprises a substrate and an image receiving coating situated on at least one surface of the substrate, said entire image receiving coating containing a biocide, and (2) causing droplets of the ink to be ejected in an imagewise pattern onto the recording sheet, thereby generating images on the recording sheet, wherein the image receiving coating comprises a quaternary acrylic copolymer latex.
- 10 15. 2. A printing process according to claim 1 wherein the biocide is present in an amount of from about 10 parts per million to about 3 percent by weight of the image receiving coating.
- 15 3. A printing process according to claim 1 wherein the image receiving coating comprises a material selected from the group consisting of poly (ethylene oxide), carboxymethyl cellulose salts, hydroxypropyl cellulose, hydroxyethyl cellulose, hydroxypropyl methyl cellulose, poly (vinyl alcohol), poly (vinyl pyrrolidone), hydroxyethyl methyl cellulose, hydroxyethyl methyl cellulose, and mixtures thereof.
- 20 4. A printing process according to claim 1 wherein the biocide is a non-ionic biocide.
- 25 5. A printing process according to claim 1 wherein the biocide is an anionic biocide.
- 30 6. A printing process according to claim 1 wherein the substrate is paper.
- 35 7. A printing process according to claim 1 wherein the substrate is a transparent polymeric material.
- 40 8. A printing process according to claim 1 wherein the printing apparatus employs a thermal ink jet process wherein the ink in the nozzles is selectively heated in an imagewise pattern, thereby causing droplets of the ink to be ejected in imagewise pattern.
- 45 9. A process according to claim 1 wherein the biocide is 5-chloro-2-methyl-4-isothiazolin-3-one, 2-methyl-4-isothiazolin-3-one, 2-(thiocyanomethylthio) benzothiazole, bis (trichloromethyl) sulfone, N-hydroxymethyl-N-methyl dithiocarbamate salts, 2-mercapto benzothiazole salts, mixtures thereof, or a mixture containing a quaternary ammonium salt and one or more of 5-chloro-2-methyl-4-isothiazolin-3-one, 2-methyl-4-isothiazolin-3-one, 2-(thiocyanomethylthio) benzothiazole, bis (trichloromethyl) sulfone, N-hydroxymethyl-N-methyl dithiocarbamate salts, or 2-mercapto benzothiazole salts.
- 50 10. A process according to claim 1 wherein the biocide is present in an amount of no more than about 25 parts per million by weight of the image receiving coating.
- 55 11. A process according to claim 1 wherein the biocide is 5-chloro-2-methyl-4-isothiazolin-3-one.
- 60 12. A process according to claim 1 wherein the biocide is 2-methyl-4-isothiazolin-3-one.
- 65 13. A process according to claim 1 wherein the biocide is 2-(thiocyanomethylthio) benzothiazole.
14. A process according to claim 1 wherein the biocide is bis (trichloromethyl) sulfone.
15. A process according to claim 1 wherein the biocide is a N-hydroxymethyl-N-methyl dithiocarbamate salt.
16. A process according to claim 1 wherein the biocide is a 2-mercapto benzothiazole salt.
17. A process according to claim 1 wherein the biocide is a mixture of a quaternary ammonium salt and one or more

**17**

of 5-chloro-2-methyl-4-isothiazolin-3-one, 2-methyl-4-isothiazolin-3-one, 2-(thiocyanomethylthio) benzothiazole, bis (trichloromethyl) sulfone, N-hydroxymethyl-N-methyl dithiocarbamate salts, or 2-mercapto benzothiazole salts.

**18.** A process according to claim 1 wherein the biocide is a mixture of a quaternary ammonium salt and bis (trichloromethyl) sulfone.

**19.** A process according to claim 1 wherein the biocide is a mixture of a N-hydroxymethyl-N-methyl dithiocarbamate salt and a 2-mercapto benzothiazole salt.

**20.** A process according to claim 1 wherein the biocide is a mixture of 5-chloro-2-methyl-4-isothiazolin-3-one and 2-methyl-4-isothiazolin-3-one.

**21.** A process according to claim 1 wherein the image receiving coating further comprises a carboxymethyl cellulose salt, polyethylene oxide, and a N-hydroxymethyl-N-methyl dithiocarbamate salt.

5

10

15

**18**

**22.** A process according to claim 1 wherein the image receiving coating further comprises a carboxymethyl cellulose salt, polyethylene oxide, a N-hydroxymethyl-N-methyl dithiocarbamate salt, and a 2-mercapto benzothiazole salt.

**23.** A process according to claim 1 wherein the image receiving coating further comprises a cationic hydroxyethyl cellulose polymer, polyethylene oxide, bis (trichloromethyl) sulfone, and a quaternary ammonium salt.

**24.** A process according to claim 1 wherein the image receiving coating further comprises hydroxypropylmethyl cellulose, 5-chloro-2-methyl-4-isothiazolin-3-one, and 2-methyl-4-isothiazolin-3-one.

**25.** A process according to claim 1 wherein the image receiving coating further comprises hydroxypropylmethyl cellulose, a carboxymethyl cellulose, polyethylene oxide, and 2-(thiocyanomethylthio) benzothiazole.

\* \* \* \* \*